

Feb. 27, 1951

M. G. DRIESSEN ET AL  
PROCESS FOR THE SEPARATION OF SOLIDS OF DIFFERENT  
SPECIFIC GRAVITY AND GRAIN SIZE  
Filed April 23, 1946

2,543,689



Maximiliaan G. Driessen, Inventor  
Centinus Krijgsman &  
Jan N. J. Leeman,  
By *Cochrane, Tracy & Rutherford*  
their Attorneys

Patented Feb. 27, 1951

2,543,689

# UNITED STATES PATENT OFFICE

2,543,689

## PROCESS FOR THE SEPARATION OF SOLIDS OF DIFFERENT SPECIFIC GRAVITY AND GRAIN SIZE

Maximiliaan G. Driessen, Brunssum, and Cen-  
tinus Krijgsman and Jan N. J. Leeman, Hoens-  
broek, Netherlands; Antje G. Driessen, admin-  
istrator of said Maximiliaan G. Driessen, de-  
ceased, assignors to De Directie van de Staats-  
mijnen in Limburg, Heerlen, Netherlands.

Application April 23, 1946, Serial No. 664,320  
In the Netherlands July 21, 1942

Section 1, Public Law 690, August 8, 1946  
Patent expires July 21, 1962

9 Claims. (Cl. 209—173)

1

The present invention relates to a new and improved process for separating solid materials of different specific gravity and different grain size into fractions.

In practice it is often necessary to separate mixtures of solid materials of different character. In the mining industry, for example, the useful parts of the hauled or hoisted product must generally be separated. For this purpose advantage is taken of the different specific gravity of the parts. For this separation according to specific gravity various processes are known. Coal and ore washeries, using the so-called float-and-sink process, are widely employed. In these washeries fluids having a true or apparent specific gravity intermediate the specific gravities of the parts which are to be separated are employed so that the parts of a lower specific gravity than that of the fluid float, while those of a higher specific gravity sink in the fluid.

The difficulty of this process is that the resultant force which acts on the particles and which in the separating vessel determines the path of a particle having a specific gravity differing only little from the specific gravity of the separating fluid, is very small. This force is also very small for very small particles of higher specific gravity (which must sink), because the resistance against motion increases as the ratio of area to volume.

Attempts have been made to remove the difficulties of a static separation by introducing currents, but this in turn introduces the difficulty that a pure separation according to specific gravity is no longer obtained, since the separation is also influenced by the dimensions of the particles. These processes call for a pre-classification in grain sizes, which is the more difficult and complicated the smaller the dimensions of the material to be separated.

It is known that a so-called cyclone of the type discussed in the article of Maximiliaan G. Driessen entitled "Cleaning of Coal by Heavy Liquids, with Special Reference to the Staatsmijnen-Loess Process" published August 1939, in the Journal of The Institute of Fuel, London, England, has a separating effect on a suspension which is treated therein. This type of action is described in an article by Eugen Feifel entitled "Zyklonentstaubung-Der Zyklon als Wirbelsenke" (Dust Extraction by Means of a Cyclone—The Cyclone as a Vortex Sink) published in the March-April 1938 issue of "Forschung auf dem

2

Gebiete des Ingenieurwesens," published in Berlin, Germany. The Feifel article states that, in a cyclone, use is made of centrifugal force, which force may be a hundred or even a thousand times greater than gravity. Such apparatus are used to separate from a suspension the solid particles which are suspended in a gas or a fluid or to thicken (concentrate) this suspension. In a cyclone the path which is traced by the particle is determined not only by the specific gravity but also by the dimensions of the particle.

In the accompanying drawing:

Figure 1 shows diagrammatically in axial section a form of cyclone such as shown in said 15 Driessen article, and

Figures 2 to 6 are graphs illustrating characteristics of separating actions.

The cyclone 10 is here shown, Figure 1, as disposed on a vertical axis. It includes a shallow 20 top cylindrical portion 11 and a lower conical portion 12. Portion 11 has a top central opening 13, and debouching into this portion at 14 is a tangential delivery conduit 15. Portion 12 has an apex opening 16 restricted by means such as 25 shown in Figure 18 of said Driessen article.

If, for instance, a suspension of loess in water is thickened with the help of a cyclone, the fraction which is discharged at the apex contains the larger particles, whereas the fraction leaving the cyclone at the opposite end contains only the smaller particles because the specific gravity of all particles is the same. If, on the contrary, a gas containing fly-ashes consisting of different 30 specific gravity and different grain size is cleaned by means of a cyclone, there is found in the dust caught at the apex besides particles of higher specific gravity, larger particles of lower specific gravity, whereas the cleaned gas, leaving the cyclone at the opposite end, contains besides the 35 very light particles, also very small particles of higher specific gravity. Only in cases where all the particles suspended in the gas are of the same grain size would a separation according to specific gravity be effected in the cyclone. The characteristic performance of a cyclone can be represented by a curve as shown in Figure 2, whereas a device separating exactly according to specific gravity can be represented by Figure 3.

A device separating exactly according to grain size, such as a screen, is represented by Figure 4. 40 In Figure 2 the particles leaving at the apex are those to the left of and above the line 17,

50

those leaving at the top being at the other side of the line. In Figure 3 the sinking particles are above line 18 and the floating particles below. In Figure 4 the particles to the left of line 18 are those held on the screen while those to the right of the line are passed.

Hitherto the cyclone could not be used to separate a mixture of solid materials of different specific gravity and different particles size.

The present invention, however, enables the characteristic performance of a cyclone to be changed in such a way that it becomes possible to separate from a mixture of solid materials of different specific gravity and different grain size a fraction consisting only of particles below or above a certain specific gravity (the specific gravity of separation). According to the invention the mixture to be separated is treated in a cyclone with so much fine material of a specific gravity higher than the specific gravity of separation, that the fraction leaving the cyclone at the apex contains practically no particles of a lower specific gravity than the specific gravity of separation.

If enough very fine particles of a specific gravity higher than the specific gravity of separation are present in the suspension the concentration of this suspension in the apex of the cyclone apparently becomes so high that the particles of a specific gravity below the specific gravity of separation, irrespective of their dimensions, are obstructed from leaving the cyclone at the apex. By these means the result is attained that the fraction discharged at the apex contains practically only particles of a specific gravity higher than the specific gravity of separation. The characteristic performance of the cyclone can now be represented as given in Figure 5.

The fraction leaving the cyclone opposite the apex now contains besides the particles of a specific gravity below the specific gravity of separation, a small part of the particles of a higher specific gravity than the specific gravity of separation. However, these are only the very small particles. According to the invention and the method described above, it is possible to obtain with the help of the cyclone besides fractions of a specific gravity above the specific gravity of separation, those fractions having a specific gravity below the specific gravity of separation. This can be effected by removing the very fine particles from the fraction which leaves the cyclone opposite the apex. A simple way for this purpose is for instance screening. This process is of particular importance for the washing of fine coal.

Figure 6 represents the above described process. Curve ABC shows the normal characteristic performance of the cyclone. By the process according to the invention, a characteristic performance along DBC is obtained. The area 20 represents the fraction which is discharged at the apex of the cyclone containing only particles above the specific gravity of separation. The fraction discharged the cyclone at the opposite end is represented by the curve DBCFA. By removing the very small particles, for instance by screening, a fraction is left which contains only particles below the specific gravity of separation, represented by area 21 (ADBE). From the fraction containing the very small particles and represented by area 22 (EBCF) the useful parts can be regained, for instance in the preparation of coal, if so desired, with a known process such as froth flotation.

The invention will be illustrated by the following example:

Raw fine coal 0-15 mm. to which loess is added in the proportion 1 part of loess to 2 parts of coal is treated with water in a cyclone having a maximum inner dia. of 200 mm. and a maximum height of 470 mm. The lighter fraction, leaving the cyclone opposite the apex is screened on  $\frac{1}{2}$  mm. and shows the following analysis:

|                         |          |           |          |          |
|-------------------------|----------|-----------|----------|----------|
| Spec. gravity up to 1.3 | 1.3-1.35 | 1.35-1.4  | 1.4-1.45 | 1.45-1.5 |
| Per cent.               | 32.3     | 20.4      | 9.1      | 7.23     |
| Spec. gravity 1.5-1.55  | 1.55-1.6 | above 1.6 |          | 5.97     |
| Per cent.               | 4.92     | 0         | 0        |          |

The analysis of the product leaving the cyclone at the apex is as follows:

|                         |          |           |          |          |
|-------------------------|----------|-----------|----------|----------|
| Spec. gravity up to 1.3 | 1.3-1.35 | 1.35-1.4  | 1.4-1.45 | 1.45-1.5 |
| Per cent.               | 0        | 0         | 0        | .595     |
| Spec. gravity 1.5-1.55  | 1.55-1.6 | above 1.6 |          |          |
| Per cent.               | 3.04     | 5.5       | 90.7     |          |

In drawing the Tromp curve the specific gravity of separation is found to be 1.54. With this small cyclone a capacity of 7.5 ton/h. washed coal is attained. Besides loess other heavy media such as fine sand, magnetite, barytes and similar materials, or mixtures of such heavy media can be used.

We claim:

1. The continuous method of separating solid particles of different specific gravity and particle size comprising feeding under pressure tangentially into one end portion of a confined circular space a suspension in a liquid of a mass of such particles to move in a cyclonic vortex within the circular space wherein centrifugal forces will be substantially in excess of gravitational forces, a portion of the mass of particles being of substantially finer size than the remainder of the particles and of a specific gravity higher than a predetermined specific gravity of separation, discharging liquid and separated particles under pressure created by said feed from two outlets coaxial of the circular space, one of the outlets opening directly from the end portion of the space which is adjacent the point of infeed while the second outlet is located at the non-infeed end of the circular space, said portion of substantially finer particles being supplied in such quantity and the discharge from the second outlet being so restricted that a concentration of the substantially finer and higher specific gravity particles will be created and maintained in a zone adjacent the second outlet of the circular space to obstruct discharge of the particles of a specific gravity lower than said specific gravity of separation from the second discharge outlet so that the fraction discharged from said first discharge outlet will contain substantially all particles of a specific gravity lower than said specific gravity of separation and the fraction discharged at the second discharge outlet will contain substantially only particles of a specific gravity higher than said specific gravity of separation.
2. A method of the character described in claim 1 wherein the suspension is fed into the base end portion of a conical circular space.
3. A method of the character described in claim 2 wherein the second discharge outlet is at the apex of the space.
4. The continuous method of separating solid particles of different specific gravity and particle size comprising feeding under pressure tangentially into one end portion of a confined circular space a suspension in a liquid of a mass of such

particles to move in a cyclonic vortex within the circular space wherein centrifugal forces will be substantially in excess of gravitational forces, a portion of the mass of particles being of substantially finer size than, and of a material foreign to, the remainder of the particles and of a specific gravity higher than a predetermined specific gravity of separation, discharging liquid and separated particles under pressure created by said feed from two outlets coaxial of the circular space, one of the outlets opening directly from the end portion of the space which is adjacent the point of infeed while the second outlet is located at the non-infeed end of the circular space, such particles of foreign material being added in such quantity and the discharge from the second outlet being so restricted that a concentration of the substantially finer and higher specific gravity particles will be created and maintained in a zone adjacent the second outlet of the circular space to obstruct discharge of the particles of a specific gravity lower than said specific gravity of separation from the second discharge outlet so that the fraction discharged from said first discharge outlet will contain substantially all particles of a specific gravity lower than said specific gravity of separation and the fraction discharged at the second discharge outlet will contain substantially only particles of a specific gravity higher than said specific gravity of separation.

5. A method of the character described in claim 4 wherein the suspension is fed into the base end portion of a conical circular space.

6. A method of the character described in claim 5 wherein the second discharge outlet is at 35 the apex of the space.

7. The method of separating solid particles of different specific gravity into fractions comprising mixing the particles to be separated with a liquid and particles of a size substantially finer than, and of a material foreign to, the bulk of the particles to be separated and having a specific gravity higher than a predetermined specific gravity of separation, feeding under pressure the resultant suspension tangentially into one end 45 portion of a confined circular space to move in a cyclonic vortex within the circular space wherein centrifugal forces will be substantially in ex-

cess of gravitational forces, discharging liquid and separated particles under pressure created by said feed from two outlets coaxial of the circular space, one of the outlets opening directly from the end portion of the space which is adjacent the point of infeed while the second outlet is located at the non-infeed end of the circular space, said portion of substantially finer particles being added in such quantity and the discharge 10 from the second outlet being so restricted that a concentration of the substantially finer and higher specific gravity particles will be created and maintained in a zone adjacent the second outlet of the circular space to obstruct discharge of the particles of a specific gravity lower than said specific gravity of separation from the second discharge outlet so that the fraction discharged from said first discharge outlet will contain substantially all particles of a specific gravity lower than said specific gravity of separation and the fraction discharged at the second discharge outlet will contain substantially only particles of a specific gravity higher than said specific gravity of separation.

25. 8. A method of the character described in claim 7 wherein the suspension is fed into the base end portion of a conical circular space.

9. A method of the character described in claim 8 wherein the second discharge outlet is at 30 the apex of the space.

MAXIMILIAAN G. DRIESSEN.  
CENTINUS KRIJGSMAN.  
JAN N. J. LEEMAN.

#### REFERENCES CITED

The following references are of record in the file of this patent:

#### UNITED STATES PATENTS

| 40 | Number    | Name      | Date           |
|----|-----------|-----------|----------------|
|    | 1,149,463 | Pardee    | Aug. 10, 1915  |
|    | 1,197,946 | Pardee    | Sept. 12, 1916 |
|    | 1,392,401 | Chance    | Oct. 4, 1921   |
|    | 1,629,182 | Stull     | May 17, 1927   |
| 45 | 2,052,004 | Remick    | Aug. 25, 1936  |
|    | 2,104,537 | Ellis     | Jan. 4, 1938   |
|    | 2,287,115 | McCluskey | June 23, 1942  |
|    | 2,364,799 | Laughlin  | Dec. 12, 1944  |